

## UNITED STATES PATENT OFFICE

2,297,986

## METHOD OF SCOURING WOOL

Ben W. Rowland and Douglas Fronmuller, Appleton, Wis., assignors to The Institute of Paper Chemistry, Appleton, Wis., a corporation of Wisconsin

No Drawing. Application September 18, 1939,  
Serial No. 295,454

4 Claims. (Cl. 8—139)

The present invention relates to an improved process for scouring wool.

Prior to the present invention there were two chief scouring methods, i. e., (1) the soap and alkali process, and (2) the solvent process. The most prevalent of the two prior art methods was the soap and alkali process utilizing as detergents water, soap and alkali for removal of the dirt, suint and grease. This process carried out in an alkaline bath at a pH of 10.5—11.0 deleteriously affected the wool fiber and its use was recognized by the art to present serious disadvantages. The other process, utilizing relatively expensive organic solvents, was not very effective and its use was generally recognized by the art as unsatisfactory and commercially impractical.

It is, therefore, the principal object of the present invention to provide an improved process for scouring wool.

Other objects will be apparent as the description hereinafter proceeds.

We have discovered a commercially practical process for effectively removing dirt, suint, grease, etc., from wool free from the above noted disadvantages. Wool, for example, treated in accordance with the present invention retains its desirable original fiber characteristics (i. e., its physical or chemical structures are not deleteriously impaired) and is much whiter and more open than wool treated by prior art processes. Physical tests, in fact, show the process of the present invention to increase desirable characteristics such as fiber elasticity, resiliency, felting qualities, etc., and decrease undesirable characteristics such as fiber elongation.

The present invention provides the art with a satisfactory means for readily obtaining improved wool fiber heretofore unavailable.

The following example will serve to illustrate the present invention:

*Example*

About 1400 pounds of wool are first made ready at the feed end of the scouring train in accordance with general practice. About 10 pounds of sodium glycercyl lauryl sulfate are next added to and dissolved in the first scouring bowl containing about 750 pounds of warm water preferably around 140°—150° F. The wool is then submerged in the sulfate scouring solution for about 1—2 minutes, washed for about 1—2 minutes each in two rinse bowls containing warm water preferably around 120°—140° F., and finally dried by any one of the customary drying procedures.

The temperature of the sulfate scouring solu-

tion for commercial purposes is ordinarily maintained around 150° F. which requires only about 1½ minutes for scouring the wool. Lower temperatures with increased scouring time, e. g., 120° F. for 3 minutes, may be employed. Scouring times may also vary with concentration as well as temperature—the optimum conditions being readily obtainable by experimental tests. For usual operating conditions scouring times of 1—3 minutes and a temperature range of 120°—150° F. are ordinarily preferred.

The pH of the scouring solution should be 3.5 to 6.5, although a pH of 4 to 6, which keeps the wool at its isoelectric point, is preferred. As the wool grease generally has a pH value of about 8, it has been found necessary in most instances to add a small amount of buffer to the scouring solution in order to keep the pH within the proper range. Compounds such as glycercyl lauryl sulfate, sodium acid sulfate or mono-sodium phosphate are representative examples of suitable buffers for use in the present invention.

In place of the sodium glycercyl lauryl sulfate used in the above example, other organic sulfates or sulfonates may be substituted therefor. We have found, for example, that sulfated unsaturated cotton seed oil acids are particularly adaptable for use in the present invention. The alkali metal salts of higher aliphatic alcohol sulfates and higher fatty acid sulfates are representative examples of other detergents suitable for use in accordance with our process. In general, any acidic organic ester or soluble salt thereof being stable against hydrolysis in acid condition and having detergent properties may be employed. These materials are available on the open market or, if desired, may be prepared by known chemical processes.

The wool treated in accordance with the present invention in the acid scouring bath has been proven by many tests to be far superior to wool treated in accordance with the prior art processes, such as the soap-alkali process. Wool, for example, treated by our improved process employing an acid scouring bath (i. e., pH 3.5—6.5) is of increased whiteness, elasticity, resiliency and tensile strength and increased resistance to abrasion. These properties are particularly important in the wool paper-making felt art.

We have also discovered that wool treated by the acid procedure and dried to a moisture content of not less than 5 per cent, possesses a marked increase in tensile strength as compared to wool treated similarly but dried to a moisture content below 5 per cent. This unique result is

just the reverse of wool treated in an alkaline scouring bath (e. g., the soap-alkali process) in that such wool dried to a moisture content of not less than 5 per cent has a lower tensile strength than the same wool dried to less than 5 per cent water. These opposite drying effects also serve to emphasize the differences in the present scouring process and the other processes available heretofore.

It will be understood that the present invention is not limited to the above illustrative examples. All modifications coming within the spirit and scope of the present invention are intended to be covered by the following claims.

We claim:

1. The method of scouring wool for effectively removing dirt, suint, grease and the like, which comprises treating wool with an aqueous aliphatic sulfate detergent bath maintained at a temperature of about 140° to 150° F. and a pH of about 4 to 6, washing the treated wool in warm water and then drying the wool so that it contains at least about 5 per cent moisture.

2. The method of scouring wool for effectively

removing dirt, suint, grease and the like, which comprises treating wool with an aqueous alkali metal glyceryl lauryl sulfate detergent bath maintained at a temperature of about 140° to 150° F. and a pH of about 4 to 6, washing the treated wool in warm water and then drying the wool so that it contains at least about 5 per cent moisture.

3. The method of scouring wool for effectively removing dirt, suint, grease and the like, which comprises treating wool with an aqueous sulfated cotton seed oil acid detergent bath maintained at a temperature of about 140° to 150° F. and a pH of about 4 to 6, washing the treated wool in warm water and then drying the wool so that it contains at least about 5 per cent moisture.

4. The method of scouring wool for effectively removing dirt, suint, grease and the like, which comprises treating wool with a buffered acidic warm aqueous organic sulfate detergent bath maintained at a pH of 3.5 to 6.5.

BEN W. ROWLAND.  
DOUGLAS FRONMULLER.